

Sept. 11, 1934.

J. H. PLUNKETT

1,972,951

WALL STRUCTURE AND LINER THEREFOR

Filed June 2, 1932



Fig. 1



Fig. 2



Fig. 3

INVENTOR.  
John H. Plunkett  
BY Samuel Stearns  
ATTORNEY.

## UNITED STATES PATENT OFFICE

1,972,951

## WALL STRUCTURE AND LINER THEREFOR

John H. Plunkett, Beverly Hills, Calif., assignor,  
by mesne assignments, to The Patent and  
Licensing Corporation, New York, N. Y., a cor-  
poration of Massachusetts

Application June 2, 1932, Serial No. 614,860

4 Claims. (Cl. 72—124)

This invention relates to a building material and to a construction in which the material is utilized. More particularly, the invention relates to waterproof sheathing material which is suitable for 5 use as a lining beneath stucco, plaster and like material.

I have found that if a sheet of felted fibrous material is saturated with a low melting point asphalt and then coated on one side only with 10 high melting point asphalt the material forms an excellent waterproofing lining for walls, ceilings, floors and the like, to which the plaster, stucco or other similar material used as an external covering can be firmly anchored.

15 Ordinary saturated felt is rather porous and in consequence thereof is capable of absorbing moisture. If stucco or plaster is applied to a sheet of saturated felt the moisture will be absorbed from the stucco or plaster by the belt and it will exert 20 sufficient suction to firmly unite the stucco or plaster thereto. By applying a coat of high melting point asphalt to that face of the sheet of fibrous material which is opposite to that to which the stucco or plaster is anchored, the sheet can 25 be made impervious to water. Besides serving as an anchoring medium for the stucco or plaster and as a waterproofing lining for the wall, the sheet which has been so saturated and coated also serves to retain the water adsorbed from the 30 stucco or plaster, thereby causing slow drying thereof with the result that setting takes place slowly, and a very firm and hard finished wall is obtained.

My invention will be more fully understood 35 from the following description in conjunction with the accompanying drawing of which;

Figure 1 is a perspective view of my novel construction with the outer layer broken away;

Figure 2 is a cross-sectional view of the construction shown in Figure 1, and

Figure 3 is an enlarged fragmentary cross-section showing my novel construction.

Referring to the drawing, the numeral 1 indicates generally the construction in accordance 45 with my invention. The numeral 2 indicates the sheet of fibrous material which has been saturated with asphalt having a melting point asphalt of from 130 to 150° F. and coated on one side only with asphalt having a melting point of 50 from 200 to 250° F. The coating of asphalt is indicated by the numeral 3.

The sheet as thus prepared may be made in any desired length and of suitable width and wound into rolls for shipment.

55 The sheets so prepared are fastened to the studding 4 of a building so that the marginal edges are in overlapping relation as indicated at 5. As will be apparent from the drawing, the sheets are fastened to the studding with the asphalt 60 coated face thereof against the studding. The

saturated face of the sheet is on the outside. After the sheets 1, have been fastened to the studding, stucco or plaster is then applied to the saturated surface of the sheets. If necessary, wire netting may be interposed between the sheets 65 and the stucco in order to more firmly hold the stucco in place.

If the sheathing in accordance with my invention is used as a liner for outside walls, the asphalt coated surface will be innermost and the 70 saturated surface will be outermost and the stucco will be anchored thereto. If the lining sheets are used beneath plaster on inside walls, the asphalt coated surface of the sheet will be outermost 75 i. e., nearest the outer walls of the structure and the saturated surface will be innermost and the plaster will be anchored thereto.

Any water or moisture which penetrates through the stucco from the outside will reach 80 only as far as the asphalt coating and be deflected outwardly again.

The material made in accordance with my invention is cheap and simple to manufacture and at the same time provides an effective moisture- 85 impervious backing sheet to which stucco or plaster can be keyed or anchored.

I claim as my invention:

1. A wall structure comprising a layer of stucco and a sheet of fibrous felted material beneath and in contact with said stucco, said sheet of 90 fibrous material being saturated with asphalt and coated with asphalt on the surface of the sheet, out of contact with said stucco.

2. A lining for stucco, plaster and similar walls comprising a plurality of overlapping sheets 95 which have been saturated with low melting point asphalt and coated on one face only with high melting point asphalt, the uncoated face being in contact with the stucco.

3. A construction for walls, floors, ceilings and 100 the like, comprising an outer layer of stucco or plaster, a layer of waterproof material beneath said outer layer and in contact therewith, said waterproofing material comprising sheets of felted fibrous material saturated with waterproofing 105 substance and coated with a film of waterproofing substance only on the surface of said sheets which is out of contact with the outer layer.

4. A construction for walls, floors, ceilings or 110 the like, comprising overlapping sheets each composed of a unitary felted fibrous sheet saturated with bituminous material, one face of which is provided with an impervious coating the opposite face being pervious to moisture, and a layer of stucco or plaster adhering directly to said pervious 115 face.

JOHN H. PLUNKETT.